

March 26, 1929.

A. LE BOUTILLIER

1,706,725

METHOD OF HEAT TREATING ARTICLES

Filed Feb. 19, 1927

Fig. 1.



Fig. 2.



Inventor  
Austin LeBoutillier  
by A. LeBoutillier. Atty.

Patented Mar. 26, 1929.

## UNITED STATES PATENT OFFICE.

AUSTIN LE BOUTILLIER, OF WESTERN SPRINGS, ILLINOIS, ASSIGNOR TO WESTERN ELECTRIC COMPANY, INCORPORATED, OF NEW YORK, N. Y., A CORPORATION OF NEW YORK

## METHOD OF HEAT TREATING ARTICLES.

Application filed February 19, 1927. Serial No. 169,472.

This invention relates to a method of heat treating articles, and more particularly to a method of heat treating thin flat articles composed of a magnetic nickel iron alloy.

5 In the manufacture of apparatus for use in telephone circuits it is necessary to provide very thin diaphragms made of a magnetic material and for this purpose thin disks of a magnetic nickel iron alloy, generally known as "permalloy" may be employed. One method of making these disks is to sever them from thin flat strips of "permalloy" which have previously been heat treated to give them desirable magnetic and 10 physical characteristics. However, it has been found difficult to heat treat the thin "permalloy" strips without causing the strips to adhere to one another and without causing them to warp or buckle so that they 15 lose their original shape.

The object of the invention is to provide a simple and effective method of heat treating thin articles.

In carrying out the object of the invention, in one embodiment thereof a plurality 25 of articles in the form of thin flat sheets of a magnetic nickel iron alloy are interleaved with a plurality of thin flat plates of silicon steel having an oxide coating on the 30 surfaces thereof. A heavy weight is then placed upon the resulting stack of articles and the articles are heated for a predetermined period of time at a high temperature, after which they are allowed to cool slowly.

35 Other objects and features of the invention will be apparent from the following detailed description taken in conjunction with the accompanying drawing, in which

Fig. 1 is a vertical sectional view of an apparatus for heat treating articles, with a portion broken away to more clearly illustrate parts therof, and

Fig. 2 is an enlarged fragmentary sectional view thereof.

45 In the accompanying drawing in which like numerals designate the same parts throughout the several views, the numeral 10 designates generally an annealing furnace by means of which the improved method 50 may be practiced. The furnace 10 comprises a bottom 11, sides 12-12, and a top 13 made of a suitable refractory material which cooperate to form an annealing chamber 14. Surrounding the chamber 14 in close prox-

imity to the bottom, sides and top thereof, 55 and enclosed within a suitable casing 16, are a plurality of heating units 15-15 which may be of any type, such as electric resistance units, well known to the art. A removable box 17 is situated within the chamber 14 and is provided with a removable cover 18, which box is designed to hold the articles to be heat treated. A flat relatively thick steel plate 20 is placed in the bottom of the box 17 and upon this plate are stacked a 60 plurality of articles 21-21 to be annealed, in the form of thin strips of a nickel iron alloy having a nickel content of more than 25%, which are interleaved with a plurality of thin flat plates 22-22 made of silicon 65 steel having an oxide coating upon the surfaces thereof which is non-adherent to the surfaces of the articles at high temperatures. A second comparatively thick flat plate 24 is placed upon the above mentioned stack of 70 articles and plates and a second stack of articles and interleaved plates are placed upon the plate 24. Any desired number of stacks of the articles and the interspersed plates may be used, the drawing showing 75 three of such stacks, and upon the top stack are placed a plurality of heavy flat plates 26-26.

The operation of the apparatus is as follows: After the articles and plates have been 80 stacked in the box 17 as described above, the cover 18 is placed upon the box 17, the loaded box placed within the chamber 14 of the annealing furnace 10 and the doors of the chamber (not shown) are closed. The heating units 15-15 are put into operation to 85 raise the temperature of the chamber and the enclosed articles to the desired temperature, which in the case of the nickel iron alloys described is within the temperature 90 range of 1650 to 1900° F. The articles are retained at the desired temperature for a predetermined period of time, depending upon the characteristics desired. For the 95 particular articles described above, one hour has proven a satisfactory heating period. After the articles are heated for the desired 100 length of time, the box 17 containing the articles is removed from the annealing furnace 10 and the articles are allowed to cool 105 slowly before being removed from the box 17.

By interleaving the articles with the

plates of silicon steel having an oxide coating on the surfaces thereof, the articles are prevented from adhering to one another at the high temperature employed in the annealing process, while the pressure exerted by the weight of the heavy plates placed upon the stacks of articles causes the articles to assume and retain the flatness desired in the finished product. It is evident, however, 10 that the process may be employed equally well with articles having irregular surfaces by providing plates 22-22 having corresponding surfaces and the weight of the plates 26-26 will then tend to retain the 15 articles in their original shape.

What is claimed is:

1. A process for heat treating articles, which consists in interleaving a plurality of the articles with a plurality of thin plates 20 having thereon a surface layer of material which is non-adherent to the articles at high temperatures, applying pressure to the resulting stack, and heating the articles.
2. A process for heat treating thin articles, 25 which consists in interleaving a plurality of the articles with a plurality of thin plates composed of a material having an oxide coating thereon, applying pressure to the resulting stack, heating the articles at a high temperature, and slowly cooling the articles.
3. A process for heat treating thin articles composed of a nickel-iron alloy, which consists in interleaving a plurality of the articles with a plurality of silicon steel plates 30 having a surface scale thereon to prevent

adherence of the articles, and heating the resulting stack to a minimum temperature of 1650° F.

4. A process for heat treating thin flat 40 articles composed of a magnetic nickel-iron alloy, which consists in interleaving a plurality of the articles with a plurality of thin flat plates of silicon steel having an oxide coating thereon to prevent adherence of the 45 articles, applying pressure to the resulting stack to maintain the flatness of the articles, and heating the articles for a predetermined period of time within the temperature range to 1650° to 1900° F. 50

5. A process for heat treating thin flat articles composed of a magnetic nickel-iron alloy, which consists in interleaving a plurality of the articles with a plurality of thin flat plates of silicon steel having an 55 oxide coating thereon to prevent adherence of the articles, applying pressure to the resulting stack to maintain the flatness of the articles, heating the articles for about one hour within the temperature range of 1650 60 to 1900° F., and slowly cooling the articles.

6. A process for annealing metallic sheets at high temperatures, which includes interleaving the metallic sheets with metallic plates having an oxide scale to prevent the 65 metallic sheets from becoming welded together, and subjecting the interleaved articles to heat.

In witness whereof, I hereunto subscribe my name this 2nd day of February, A. D. 70 1927.

AUSTIN LE BOUTILLIER.